

# United States Patent Office

3,346,378

Patented Oct. 10, 1967

1

3,346,378

## COBALT BASE ALLOYS

Allan D. Foster, Schenectady, and Chester T. Sims, Ballston Lake, N.Y., assignors to General Electric Company, a corporation of New York  
No Drawing. Filed Mar. 22, 1965, Ser. No. 441,831  
11 Claims. (Cl. 75—171)

### ABSTRACT OF THE DISCLOSURE

High temperature oxidation and corrosion resistant cobalt base alloys useful in high temperature operating equipment have a percent by weight content consisting essentially of carbon 0.10 to 0.60, chromium 24.0 to 35.0, tungsten 6.0 to 9.0, nickel 8.5 to 11.5, iron 6.0 maximum, boron 0.50 maximum, yttrium 0.01 to 1.0, manganese 1.0 maximum as impurity, with the remainder essentially cobalt.

This is a continuation-in-part of application Ser. No. 415,507 filed Dec. 2, 1964. The invention relates to new and useful alloys. More particularly, it relates to alloys which possess suitable high temperature strength and are resistant to oxidizing, sulfidizing and other corrosive combustion gases at elevated temperatures.

It is well known that machinery depending upon the driving force of combustion gases, such as gas turbines, operate more efficiently and with greater power output at elevated temperatures. It is also well known that at such elevated temperatures the strength of many materials often decreases drastically and that they tend to become subject to excessive corrosion caused by oxidizing, or other corroding constituents in the atmospheres or fuels burned. Such constituents could be sulfur, sodium vanadium, and others. As the operating temperature of such equipment rises, relatively small improvements in the corrosion resistance and strength of such materials become important. In gas turbines operating at average temperatures of the order of about 1600° F. with peak temperatures up to about 2000° F., an improvement of only one hundred degrees Fahrenheit in the corrosion resistance of the materials of construction represents a notable advance. For example, in a typical gas turbine an increase in operating temperature from about 1500° F. to about 1600° F. represents an increase in output power of about 14% and an increased efficiency of one to five percent. It is, therefore, a principal object of this invention to provide new and useful alloys which will permit substantial increases in the operating temperatures of such equipment as gas turbines. Another object of the invention is to provide improved materials of construction for other high temperature equipment subjected to oxidizing and/or corrosive atmospheres such as furnaces and the like.

Briefly, there are provided by the present invention high-temperature corrosion-resistant cobalt-base alloys having percent by weight content of carbon 0.10 to 0.60, chromium 24.0 to 35.0, tungsten 6.0 to 9.0, nickel 8.5 to 11.5, iron 6.0 maximum, boron 0.050 maximum, yttrium 0.01 to 1.0, manganese 1% maximum as impurity not to be added, with the remainder cobalt except for incidental impurities such as phosphorus, sulfur, silicon and the like. It has been found that alloys having the above carefully controlled metallurgical composition are characterized by substantial increases in corrosion resistance, while at the same time retaining suitable rupture strength and ductility for high temperature operation. The materials are also particularly useful in that they are readily weldable, permitting the fabrication of various shaped structures.

Not only has it been found that compositions as above

2

containing from about 24 to 26.5% chromium, along with the other stated materials particularly including yttrium, are salutary in their character, but it has also been unexpectedly found that such alloys containing from about 26.5 to 35% chromium are most useful in the present respect. This is directly contrary to the teaching of the prior art which teaches that alloys having a chromium content of over about 25% by weight show an increase in scaling or deterioration at elevated temperatures. This prior art teaching is set forth, for example, in Journal of the Electrochemical Society, volume 103, No. 8, by Pfalnikar et al., entitled, "High Temperature Scaling of Cobalt-Chromium Alloys." It will thus be seen that the present invention produces results which are unexpected not only with respect to the lower ranges of chromium content, but as well for higher ranges of chromium content which proceeds directly in the face of the prior art teaching. The present invention also provides additional improvements over those conferred by 20 yttrium additions alone.

As pointed out above, the present compositions comprise a carefully formulated combination of constituents, each of which contributes to the desirable characteristics obtained. Deviations in the proportions of the materials 25 destroy this critical balance, and result in materials which have been found to be wanting in essential characteristics. For example, when the carbon content is lowered beyond that prescribed, an undesirable loss of strength results. On the other hand, increasing the carbon content 30 above that stated detracts from the weldability of the material, as well as rupture ductility, and lowers the oxidation resistance. Reduction of the chromium content below that set forth results in a detrimental loss of oxidation resistance. The nickel, iron and tungsten additives 35 do not appear to be particularly critical for oxidation and corrosion resistance but it has been found desirable to have them present in the stated ranges for suitable mechanical properties. Boron imparts ductility to the alloy where required. Increasing the boron content 40 beyond that set forth causes detrimental low-melting phases to form in the alloy. Yttrium, when used in lower amounts than that set forth above, results in a decreased oxidation resistance. As a practical matter, amounts of yttrium greater than the upper prescribed limit are difficult to 45 retain effectively through melting into the product. The cobalt base, of course, is well known for its contribution to sulfidation and oxidation resistance. Manganese can be tolerated in amounts up to about 1.00%, but it is not intentionally added in any case. Other impurities, such as 50 phosphorus and sulfur, are held to a maximum of about 0.04% each.

The following examples will illustrate the practice of the invention, it being realized that they are exemplary only and not to be taken as limiting in any way.

55

### Example 1

There was prepared an alloy consisting of, by weight 60 percent from analysis of the cast sample, carbon 0.22, chromium 24.4, nickel 10.8, tungsten 7.7, iron 1.2, boron 0.0066, yttrium 0.15, manganese 1.02, with about 0.007 of phosphorus and 0.009 sulfur as impurities with the remainder essentially cobalt. This alloy was cast into 65 pieces having dimensions of 1 1/4 inches diameter by 5 inches long from which one inch diameter discs 0.060 inch thick were cut for testing, and compared with a typical prior art alloy having a percent by weight content of carbon 0.23, chromium 25.5, nickel 10.5, tungsten 6.9, iron 0.82, boron 0.007, with 0.54 manganese, 0.02 each 70 of phosphorus and sulfur as impurities and with the remainder essentially cobalt. It will be noted that this prior

art alloy is lacking in yttrium, which it has been found imparts unexpected and advantageous qualities to the present alloy.

When test pieces of the material of the above example and the above prior art material were tested edgewise to the combustion gas stream flow in a small burner apparatus at a temperature of 2000° F. burning natural gas with an air-to-fuel weight ratio of 50 to 1, the corrosion in mils per side of the prior art material after 594 hours was 14.6. On the other hand, the material of the above example had corresponding corrosion of only 5.7 mils per side. After 984 hours the prior art material exhibited corrosion of 20.4 mils per side and after even 2431 hours the material of Example 1 exhibited corrosion of only 15.9 mils per side. It will thus be seen that the present above alloy exhibits about a three-fold increase in oxidation resistance at 2000° F. The material of the above example was tested under sulfidizing conditions, as was the above prior art material, in a test burner operating at a temperature of 1600° F. with an air-to-fuel weight ratio of 68 to 1, burning a distillate oil containing 3.8% by weight of sulfur to which 325 arts per million of sodium chloride had been added. In this type of test, deposition of molten material can occur on the leading edge of the test specimen, causing a higher penetration rate than where the deposition does not occur. The data presented here are both the minimum attack (no molten deposition) and the maximum attack where molten material resided. After 465 hours of such testing, the typical prior art material had a corrosion in mils per side of the test specimen ranging from about 3.8 (minimum) to 18.1 mils (maximum). On the other hand, the material of Example 1, even after 584 hours of operation under such rigorous conditions, had only about 1.8 (minimum) to 6.9 mils (maximum) per side of corrosion.

As pointed out above, not only are the alloys of the present invention characterized by good oxidation and sulfidizing resistance, but their fabrication into various shaped structures is facilitated by the fact that they are readily weldable.

The rupture strength of the material of Example 1 at 10<sup>3</sup> hours at a temperature of 1600° F. is about 10,500 p.s.i., which is the same value obtained from prior art material. The rupture ductility of the above exemplary material also compares favorably with prior art material.

Example 1 was repeated in all respects except for the alloy constituent content and the alloys tested as shown in the table below:

the notable advance in corrosion resistance. The rupture ductility of the materials represented in the table also compares favorably with prior art material.

There are provided, then, by the present invention, new and useful alloys which are particularly characterized by their high strength at elevated temperatures and their ability to withstand at such elevated temperatures corrosive attack as from oxidizing and sulfidizing combustion gas constituents. They are particularly useful for fabricating gas turbine parts such as nozzle partitions, as well as parts of other equipment which are exposed to high temperature corrosive and/or oxidizing conditions. They are also useful in general in furnaces for fans, runners, and in other equipment which operate under similar rigorous conditions.

What we claim as new and desire to secure by Letters Patent of the United States is:

1. A high temperature resistant alloy consisting essentially of by weight carbon 0.10 to 0.60 percent, chromium 24.0 to 26.5 percent, tungsten 6.0 to 9.0 percent, nickel 8.5 to 11.5 percent, boron 0.050 percent maximum, yttrium 0.01 to 1.0 percent, iron 6.0 percent maximum with the remainder essentially cobalt.

2. A high temperature resistant alloy consisting essentially of by weight carbon 0.22 percent, chromium 24.4 percent, tungsten 7.7 percent, nickel 10.8 percent, boron 0.0066 percent, yttrium 0.15 percent, iron 1.2 percent, with the remainder essentially cobalt.

3. A high temperature resistant alloy consisting essentially of by weight carbon 0.10 to 0.60 percent, chromium 24.0 to 35.0 percent, tungsten 6.0 to 9.0 percent, nickel 8.5 to 11.5 percent, boron 0.050 percent maximum, yttrium 0.01 to 1.0 percent, iron 6.0 percent maximum, with the remainder essentially cobalt.

4. A high temperature resistant alloy consisting essentially of by weight carbon 0.10 to 0.60 percent, chromium 26.5 to 35.00 percent, tungsten 6.0 to 9.0 percent, nickel 8.5 to 11.5 percent, boron 0.050 percent maximum, yttrium 0.01 to 1.0 percent, iron 6.0 percent maximum with the remainder essentially cobalt.

5. A high temperature resistant alloy consisting essentially of by weight carbon 0.23 percent, chromium 28.9 percent, tungsten 8.4 percent, nickel 10.4 percent, boron 0.001 percent, yttrium 0.05 percent, iron 0.65 percent, with the remainder essentially cobalt.

6. A high temperature resistant alloy consisting essentially of by weight carbon 0.24 percent, chromium 29.6 percent, tungsten 8.4 percent, nickel 10.4 percent, boron

TABLE

| Ex.    | Composition (Wt. percent) <sup>1</sup> Chemical Analysis |      |      |      |     |      |      |        |                         | Oxidation-Corrosion, 2,000° F. |                      | Stress-Rupture Behavior      |                         |                             |
|--------|----------------------------------------------------------|------|------|------|-----|------|------|--------|-------------------------|--------------------------------|----------------------|------------------------------|-------------------------|-----------------------------|
|        | C                                                        | Cr   | Y    | Ni   | W   | Fe   | Mn   | B      | Co                      | Time, Hrs.                     | Corrosion, mils/side | Rupture Strength, p.s.i.     | Temp., ° F.             | Time to Failure, Hrs.       |
| 2----- | 0.23                                                     | 28.9 | 0.05 | 10.4 | 8.4 | 0.65 | 0.40 | 0.0010 | Bal. <sup>2</sup> ----- | 635                            | 5.9                  | { 20,000<br>10,000<br>5,000  | 1,450<br>1,600<br>1,800 | 331.4<br>1,726.0<br>1,490.8 |
| 3----- | 0.24                                                     | 29.6 | 0.38 | 10.4 | 8.4 | 0.70 | 0.41 | 0.002  | Bal. <sup>2</sup> ----- | 635                            | 4.5                  | { 20,000<br>10,000<br>20,000 | 1,450<br>1,600<br>1,450 | 505.3<br>1,075.6<br>409.1   |
| 4----- | 0.24                                                     | 28.6 | 0.39 | 10.5 | 8.3 | 0.66 | 0.41 | 0.0011 | Bal. <sup>2</sup> ----- | 609                            | 4.9                  | { 10,000<br>20,000<br>10,000 | 1,600<br>1,450<br>1,600 | 970.4                       |
| 5----- | 0.26                                                     | 31.0 | 0.17 | 8.5  | 7.9 | 0.72 | 0.29 | 0.0025 | Bal. <sup>2</sup> ----- | (4)                            | (4)                  | { 15,000                     | 1,600                   | 35.2                        |

<sup>1</sup> Lesser constituents and impurities from common starting materials about as follows: Phosphorous 0.02 wt. percent.

<sup>2</sup> Balance essentially cobalt.

<sup>3</sup> About.

<sup>4</sup> Not tested.

From the above table it will be noted that compositions of the present invention containing relatively higher amounts of chromium produce alloys which exhibit exceptionally good corrosion-resistance at elevated temperatures. It will also be noted that the stress-rupture behavior as set forth is equivalent to prior art material, even with

about 0.002 percent, yttrium 0.38 percent, iron 0.70 percent, with the remainder essentially cobalt.

7. A high temperature resistant alloy consisting essentially of by weight carbon 0.24 percent, chromium 28.6 percent, tungsten 8.3 percent, nickel 10.5 percent, boron 0.0011 percent, yttrium 0.39 percent, iron 0.66 percent, with the remainder essentially cobalt.

8. A high temperature resistant alloy consisting essentially of by weight carbon 0.26 percent, chromium 31.0 percent, tungsten 7.9 percent, nickel 8.5 percent, boron 0.0025 percent, yttrium 0.17 percent, iron 0.72 percent, with the remainder essentially cobalt.

9. A high temperature resistant structure comprising the alloy of claim 1.

10. A high temperature resistant structure comprising the alloy of claim 3.

11. A high temperature resistant structure comprising the alloy of claim 4.

## References Cited

## UNITED STATES PATENTS

|           |         |               |       |        |
|-----------|---------|---------------|-------|--------|
| 2,744,010 | 5/1956  | Callaway      | ----- | 75—171 |
| 2,746,860 | 5/1956  | Binder et al. | ----- | 75—171 |
| 2,855,295 | 10/1958 | Hansel        | ----- | 75—171 |
| 2,996,379 | 8/1961  | Faulkner      | ----- | 75—171 |
| 3,202,506 | 8/1965  | Deutsch       | ----- | 75—171 |

HYLAND BIZOT, *Primary Examiner.*

RICHARD O. DEAN, *Examiner.*